

Aug. 9, 1932.

C. A. CADWELL

1,871,257

WELDING ELECTRODE

Filed Oct. 19, 1925



INVENTOR.  
*Charles A. Cadwell*  
BY  
*Fay, Oberlin & Fay*  
ATTORNEYS.

## UNITED STATES PATENT OFFICE

CHARLES A. CADWELL, OF CLEVELAND HEIGHTS, OHIO, ASSIGNOR TO THE ELECTRIC RAILWAY IMPROVEMENT COMPANY, OF CLEVELAND, OHIO, A CORPORATION OF OHIO

## WELDING ELECTRODE

Application filed October 19, 1925. Serial No. 63,299.

The present improvements, relating, as indicated, to metallic electrodes, have more particular regard to coated metallic pencils (rods or wires) of the type used in arc welding.

It has been the practice for some time in metal working by electricity to employ what are known as coated metallic pencils in order either to introduce alloying and reducing ingredients into the weld or to secure certain other desirable results in the manipulation of the pencil. For example, a bare metallic pencil or electrode if not carefully handled is apt to stick to the work with consequent damage and delay. Accordingly, the coatings heretofore used have been composed of materials that when highly heated form a slag adapted to protect the metal of the weld from oxidation and from too rapid chilling, and such materials have also been selected with a view to their insulating character, which is of value to the operator in certain cases. Asbestos and chalk are examples of the materials just referred to. The purpose in employing an alloying or reducing agent in the coating is of course obvious and this has been introduced, for example, in the form of a fine wire interwoven with the material of the coating or of a metallic powder added to such material.

The object of the present improved coating is to overcome difficulties of a different character, for the meeting of which none of the coatings heretofore employed or proposed, so far as I am aware, is suited. To this end I employ a composition differing radically from any heretofore employed in coatings of the type in question. For example, instead of an insulating material, I employ one that is a fairly good conductor even when cold. Furthermore, the coating instead of melting at a temperature lower than that of the metal of the electrode, melts at a higher temperature and so tends to assume the form of an annular extension or sleeve that projects beyond the point of the electrode so as to retard the deposition of metal and generate a higher temperature to a corresponding greater penetration or depth of weld. Furthermore, the coating material in-

cludes an ingredient which under the heat of the arc is decomposed into a reducing element or elements which react with the metal of the weld to overcome oxidation and to improve the quality of such metal.

To the accomplishment of the foregoing and related ends, the invention, then, consists of the ingredients and resultant coated product hereinafter fully set forth and particularly pointed out in the claims, the annexed drawing and the following description setting forth in detail but several of the various ways in which the principle of the invention may be utilized.

In said annexed drawing:—

Fig. 1 is a side elevation and partial central section of an electrode as coated in accordance with the present invention; Fig. 2 is a similar view of such electrode as it appears in use when connected on the positive side; and Fig. 3 is a similar view of such electrode as it appears in use when connected on the negative side.

The invention will be first described with particular reference to coated copper arc weld pencils such as are employed, for example, in certain known methods for attaching copper bonds to steel rails. In such case, a bare metallic copper electrode deposits metal in large globules which fall intermittently from the point of the electrode and which amalgamate with each other only in case the temperature of the work is high enough to prevent a chill of the first drop before the next shall have fallen. Inasmuch as copper is a metal of relatively low melting point, a chilled or cold shot condition is always found at the bottom of a copper arc weld made with bare pencil. Particularly is this true in the application of this method of welding to rail bonding, where the first drops from the copper electrode may fall on the cold copper of the conductor.

Even if a mold or dam be used in an effort to puddle the mass of the metal deposited into a molten lake, the critical part of the weld, that is, the contact, where the first metal from the electrode falls, will show the well known cold shot weakness. If the bare copper electrode is used to deposit metal in

strings or layers, as for instance on top of the lower flange of a rail, the mass deposited will be found to resemble a conglomerate of nodules poorly bonded together.

- 5 The difficulties attending the use of a bare copper electrode for rail bonding, resulting from cold shot effect, are greatly increased by the condition of the surface of the rail to be bonded. Any reducing agent introduced as an alloy into the copper metal of the electrode, capable of reacting with the oxide found on the surface of the average rail, requires more heat for a good reaction than can possibly be obtained from the cold shot metal 70
- 10 dropped intermittently from a bare copper electrode, although it must be said that the chilling effect of a steel body is much less than one of copper and that on a comparatively clean rail, copper arc metal from a 75
- 15 bare electrode makes better contact with the steel than it does with the copper of the bond conductor. The greatest difficulty from poor rail contact in using a bare copper electrode results from an adverse polarity. The 80
- 20 common practice on electric railways of using trolley current direct through a rheostat, without transformation, for bonding, dictates that a positive electrode be used on track rail and a negative electrode on third 85
- 25 rail. The greatest difference exists in the action of a bare copper electrode in the two cases. A drop of metal falling from the end of a positive electrode drops downwards, while from the end of a bare negative pencil, 90
- 30 working on third rail, the drops of metal are propelled with force by a flickering, fitful arc flame that sends the successive drops in unexpected directions. 95
- 35 As previously indicated, I have discovered 100
- 40 that if there be applied a coating to such a copper welding pencil, which is not only an agent for the reduction of any oxides of iron or copper that might occur at or in the weld, but which under the action of the arc becomes 105
- 45 a plastic tube encasing the copper at the point of the electrode and draws somewhat over the point like a glass tube softened by heat for sealing, not only is the actual welding operation facilitated, but a much 110
- 50 more homogeneous juncture is obtained between the parts being welded together, e. g. bond and rail. By employing for this coating a material that not only becomes thus 115
- 55 plastic upon heating, but is also a good conductor with a melting point considerably higher than copper, the deposition of molten copper is greatly retarded with a corresponding increase in the amount of heat introduced 120
- 60 into the weld. In fact, the action of this coated pencil is more that of an ideal self-feeding, non-metallic arc, under which the molten copper is deposited more as a continuous spray of highly superheated metal than 125
- 65 as a succession of the large drops from a

bare metallic electrode. The absence of large drops and a spraying action as from an atomizer results from the constricted, plastic and overshot envelope of the electrode end which exercises a capillary attraction for the 70 molten metal before it can collect in large drops, and also from the volatilization of certain elements in the coating which help to break up metallic globules.

The thickness and composition of the coating may be varied to secure any degree of heat, with accompanying slower rate of deposition desired, the limit being a coating so refractory that after the first few drops of copper have fallen, the end of the copper rod 75 will have retreated to a distance above the end of the electrode, which end, from the material of the coating alone, becomes a very stable non-metallic electrode, with the result 80 that no more, or very little, copper will fall 85 and only a heating arc will remain.

I have found that carborundum or silicon carbide, SiC, constitutes, when subjected to the action of the arc flame, a satisfactory material for the reduction of the oxides that 90 occur in welding and at the same time prevents oxidation from the air and insures a sound set in the copper deposited. This compound or material also introduces elements for deoxidation which, if they occur in excess 95 of oxidation needs, will alloy with both the copper and steel of the weld, while such material is also a conductor of the current of the arc and thus when the coating projects as an overshot envelope at the end of the electrode, 100 it will carry the current where the heat intensity is greatest and thus retard the flow of metal and consequently introduce more heat into the weld. Finally, it is refractory 105 under heat with a melting point considerably above that of the ordinary metals.

In order to impart to the coating composition a plastic condition when it approaches the melting point, so that it will not fall off 110 in crumbs, it is desirable to admix with such silicon carbide a binding material such as high silica clay, in which the binding quality is developed by the addition of water.

It is also desirable to include in the composition a certain amount of volatile matter to assist in breaking up large globules of molten metal as well as provide a fluid slag for floating off refractory crumbs, and for this purpose the fusible silicates comprised 115 in common bottle glass, for example, may be added to the clay binder.

Finally, in order that the composition may be quickly and cheaply applied to the metallic pencil and be secured against dislodgment from handling, a suitable water soluble gum is added, a relatively small quantity of this in combination with the clay binder being sufficient for the purpose. The following is 120

typical of a satisfactory composition including the ingredients named above, viz:—

|                   | Per cent |
|-------------------|----------|
| Silicon carbide   | 68.5     |
| Clay              | 10.5     |
| Fusible silicates | 16.5     |
| Gum               | 4.5      |

The foregoing percentages are based on the weight of the materials when dry, the materials being mixed in this condition and then made into a thin paste by the addition of water and applied to the rod or pencil with a brush. After drying a coat of varnish may be added to toughen the skin of the coating. In the process of welding the varnish and gum both burn away in advance of and without disturbing the high temperature bond due to the clay, so that the coating will persist and subserve the functions hereinbefore described.

The foregoing improved coating works very well either on the positive or negative side, i. e. whether the current flows from the work to the electrode, or vice versa. There is, however, a distinction to be noted in the form of the arc as it attaches to the point of the electrode in the one case or the other. Thus, as shown in Fig. 2, where the electrode is on the positive side, the adjacent portion of the arc is more or less confined to the exposed end of the metallic pencil, while, as shown in Fig. 3, where the electrode is on the negative side, the arc assumes a more spreading form and attaches to the projecting coating envelope as well as to the end of the metallic pencil; however, such envelope tends to close more or less across such end. In both cases the metal will lie back of the end an appreciable distance and will always present a clean appearance when the arc is discontinued, showing that there is no tendency for the metal to oxidize before it is deposited.

In case the deposition of the metal is unduly retarded, the projecting envelope or the outer portion thereof may be readily broken off by lightly striking the same against the parts being welded; while, on the other hand, if a coating of sufficient thickness is employed, by proper manipulation the arc may be struck entirely from such projecting envelope portion and used as a cutting arc.

While the melting point of iron or steel is considerably higher than that of copper, the temperature at which the envelope will melt is still higher and substantially the same operative results are obtained where my improved coating is used on such iron or steel pencil as with a copper pencil. Obviously it may be employed with equal advantage as a coating for pencils composed of other metals or alloys having the same relationship in the matter of temperature of fusion.

Other modes of applying the principle of

my invention may be employed instead of the one explained, change being made as regards the materials employed, provided the ingredients or elements stated by any of the following claims or the equivalent of such stated ingredients or elements be employed.

I therefore particularly point out and distinctly claim as my invention:—

1. An electrode for electric arc welding, which comprises a copper containing metallic rod and an envelope thereon containing silicon carbide in substantial proportion.

2. An electrode for electric arc welding, which comprises a copper containing metallic rod and an envelope thereon containing about 68 per cent of silicon carbide.

Signed by me, this 13th day of October, 1925.

CHARLES A. CADWELL.

85

90

95

100

105

110

115

120

125

130